

## UNITED STATES PATENT OFFICE

2,147,645

PROCESS FOR THE PRODUCTION OF  
METALLIC MAGNESIUM

Daniel Gardner, Rueil-Malmaison, France, assignor to Studien- & Verwertungs-Aktiengesellschaft, Neuhausen, Switzerland, a joint-stock company of Switzerland

No Drawing. Application July 29, 1936, Serial No. 93,177. In Great Britain December 23, 1935

10 Claims. (Cl. 75—67)

This invention relates to processes for the production of magnesium, being concerned with the industrial production of this metal, reference to which is intended to include alloys thereof.

5 Heretofore magnesium has been mainly obtained by the electrolysis of magnesium chloride produced from magnesium ores. A number of electrolytic processes for the production of magnesium in this manner have been proposed, but one 10 of the main difficulties that is experienced in all electrolytic processes is that of removing from the magnesium the last traces of chlorides which remain occluded in the metal.

The present invention has for its object to 15 produce, by a non-electrolytic process, magnesium cheaply and of a high degree of purity from any magnesium ores or compounds of commercial value.

Already in 1867 Parkinson (Journal of the 20 Chemical Society, Vol. V, p. 127) described the direct production of magnesium sulphide by heating magnesium filings with sulphur or sulphur vapours; hereby a hard brittle difficultly fusible mass of impure magnesium sulphide is 25 obtained. When obtained by indirect methods from magnesium compounds, magnesium sulphide is an unstable body which readily undergoes decomposition on exposure to air and still more moisture, whereby magnesium hydroxide is 30 formed. Further, the formation of magnesium sulphide, which is of an endothermic character by prior methods takes place rather slowly.

It is to be stated, that Geelmuyden (Comptes Rendus vol. 130 of 1900, page 1029) when working 35 on the reduction of certain sulphides by calcium carbide, has found that a mixture of magnesium sulphide (prepared by the action of hydrogen sulphide on anhydrous magnesium sulphate) and calcium carbide was heated for five 40 minutes in a carbon tube with a current of 850 amperes at 45 volts, luminous flames were observed during the heating process proving volatilization of magnesium.

Magnesium sulphide as previously obtained by 45 the direct action of sulphur on magnesium or by various indirect methods heretofore employed has not hitherto found any industrial application as a starting product for the manufacture of magnesium, but if special precautions be observed, in its manufacture, magnesium sulphide is easily obtainable and, under appropriate conditions as will be hereinafter described, is a very suitable product for the manufacture of magnesium.

50 According to the present invention a process

for the production of magnesium from magnesium ores or compounds consists in first producing magnesium sulphide by heating a magnesium compound, such as magnesia, with a carbonaceous reducing agent in sulphur vapours 5 and/or a gaseous or vaporized non-metallic sulphur compound, such as carbon bisulphide or sulphuretted hydrogen, or without a carbonaceous reducing agent in vapours of carbon bisulphide, to a temperature sufficiently high, say within the 10 range of about 800°—1200° C. or over, to convert the bulk of the magnesium compound treated into magnesium sulphide, this reaction being carried out in an atmosphere substantially free from moisture, oxygen and air, and then sub- 15 jecting the magnesium sulphide so formed to reduction by heating it with a carbide of an alkali earth metal, preferably calcium carbide, in an atmosphere of a reducing and/or inert gas and in the substantial absence of moisture, nitrogen 20 and oxygen or oxygen-containing gases.

The reduction of the magnesium sulphide by calcium carbide takes place according to following equation:



In order to obtain a good yield of magnesium, it is essential to use the magnesium sulphide and the carbide in a fine state of subdivision and the reaction is effected in a gaseous atmosphere at 30 normal or at reduced pressure.

Since magnesium sulphide readily undergoes decomposition on exposure to air and moisture, it is desirable to use it immediately for the reduction to metal, but if it is not so used the magnesium sulphide should be stored free from moisture in hermetically sealed receptacles.

A good yield of magnesium and a quick reaction are obtained by introducing into the mixture of finely ground magnesium sulphide and carbide a suitable flux, such as a chloride or a fluoride, the boiling point of which is above that at which magnesium distills. As fluxes suitable for their purpose there may be mentioned for instance anhydrous calcium chloride or a mixture of anhydrous calcium chloride and aluminum fluoride.

If no flux is added to the mixture it is advisable to come up in temperature for the reduction, say up to 1500°—1600° C.

The mixture of magnesium sulphide and carbide, with or without a flux, is introduced into the heated zone of a furnace, in which the decomposition of the sulphide according to the above equation is effected. The temperature of 50 55 60

the heated zone must be preferably so chosen that the magnesium produced can be easily removed from the mixture by distillation. As the magnesium distills under normal pressure at 5 about 1120° C., it is suitable to choose a temperature above this point, say 1200° or 1250° C. It is of course possible to choose a higher temperature if required; when working under reduced pressure the temperature can be some- 10 what lower.

The magnesium vapours coming from the reduction chamber are entered into special condensing chambers where they can be directly cooled and obtained in the molten or solid state.

15 In carrying out the process, the magnesium is collected at normal pressure, in an atmosphere of hydrogen and/or an inert gas, such as argon or helium, or another gas which has no action on magnesium, for example a gaseous hydrocarbon 20 such as methane.

If desired the collected magnesium can be directly combined with other metals such as for example aluminium or beryllium to form magnesium alloys.

25 The reduction of the magnesium sulphide to metal is an exothermic reaction which takes place rather more energetically as compared with the known reduction of magnesium oxide by calcium carbide, as mentioned in the French patent of 30 Matignon No. 488,735.

The reduction as suggested in the present invention can be so regulated that a continuous action takes place; for this purpose, when the process is carried out under normal pressure, it 35 is suitable to maintain in the reaction zone of the reduction furnace a temperature of 1200°-1300° C., for instance 1250° C. As stated above magnesium thus obtained distills under normal pressure at about 1120° C., and can be continuously collected in a condensing chamber or, if desired, it may be directly introduced into a bath of molten metal in the condensing chamber in order to produce an alloy of magnesium.

If the reaction is carried out in the absence of 45 a flux, it may be advisable to considerably raise the temperature over 1300° C. Interesting results are obtained for instance at a temperature of about 1600° C. without a flux; it is however preferable to work at about 1250° C. whilst using 50 a flux.

In carrying out the present process for the reduction of the magnesium sulphide and the distillation of magnesium, care must be taken to obtain the residual slag in the form of a dry mass 55 which can be continuously removed from the furnace in which the reaction is effected, for instance by means of a worm conveyor. It is more difficult to remove a tacky slag; therefore the formation of a tacky slag must be avoided as its 60 removal would create difficulties.

It is desirable to provide a filter or a screen for the magnesium vapours; such filters can suitably take the form of a graphite screen, which is located at the end of the furnace chamber (re- 65 duction chamber) just in front of the outlet conduit therefrom, through which the magnesium vapours pass into the condensing chamber.

The production of the magnesium sulphide which is used in the present process for obtaining 70 the metal can be effected by heating a magnesium compound, with or without a carbonaceous reducing agent, with sulphur vapours and/or a gaseous or vaporised non-metallic and non-oxygen-containing sulphur compound to a tem- 75 perature sufficiently high, for example about 800°

to 1200° C., to convert the magnesium compound treated into magnesium sulphide, the reaction for the formation of the magnesium sulphide being carried out in an atmosphere free from moisture, oxygen and air.

In making the magnesium sulphide the necessary conditions can be realised by effecting the formation of the magnesium sulphide in the presence of sulphur vapours, sulphuretted hydrogen or derivatives thereof, carbon bisulphide 10 in a reducing atmosphere such as hydrogen or hydrocarbons, or an inert gas such as argon or helium, care being taken that all the reagents and the atmosphere in which the reaction is effected are freed from moisture and air.

15 Where the atmosphere in which the reaction is carried out comprises hydrogen, it is to be observed that the hydrogen functions only as a reducing atmosphere, since hydrogen has no action either in the formation of the magnesium sulphide (for example from magnesium sulphate) or on the sulphide once the latter has been formed.

The formation of the sulphide takes place at a 20 temperature of about 800° C. when carbon bisulphide is used. By producing the magnesium sulphide starting from magnesite calcined at low temperature (for instance 600°-800° C.), sulphur and charcoal (or shale, turf or lignite) the reaction temperature is suitably raised up to about 25 950° C. If ordinary coke were used as carbon containing material, it would be necessary to work at a higher temperature, say at about 1200° C.

Once the anhydrous magnesium sulphide has 30 been formed, it is then reduced to metal, this 35 being effected according to the present invention by a carbide, preferably calcium carbide, in the manner already described more in detail.

It is to be observed that the first reaction in the present process, that is to say the formation 40 of the magnesium sulphide, is an endothermic one and requires a somewhat lengthy time for its completion, whereas the second reaction in the process namely the reduction of the magnesium sulphide to metal, is an exothermic reaction which takes place rather energetically as 45 compared with the known reduction of magnesium oxide by calcium carbide.

The production of the magnesium sulphide may 50 be carried out in any suitable furnace, such as a tubular furnace provided with a suitable refractory lining. The lining may be made from fused magnesia, graphite or other materials resistant to vapours of sulphur or sulphur compounds at the hereinbefore mentioned high temperatures. 55 The outlet end of the furnace in which the reaction for the production of the magnesium sulphide is effected, is suitably connected with a condensing chamber, the end of said chamber being for instance closed by a suitable stopper 60 made of refractory material. For continuous working the magnesium sulphide should be continuously removed from the furnace.

After the magnesium sulphide has been formed 65 there is mixed with it in the furnace chamber the requisite quantity of powdered calcium carbide and powdered flux, whereby, at the high temperature prevailing, decomposition of the sulphide with liberation of the metal is effected.

The present process is applicable to various 70 magnesium ores and compounds, but it will of course be understood that the precise method employed for the formation of the magnesium sulphide will vary according to the nature of the 75

particular magnesium ore or compound treated.

Magnesium sulphide hitherto obtained by direct action of sulphur and magnesium (Parkinson) or by various indirect methods has not found any industrial application as yet as a starting product for the manufacture of magnesium.

It may also be mentioned that products, such as sulphur or carbon bisulphide, employed in the present process in the formation of the magnesium sulphide can be recovered for reuse in the process.

The following are some examples for the manufacture of magnesium by the new process according to the present invention.

#### 15 EXAMPLE 1

##### *Production of magnesium from magnesia*

The powdered magnesium oxide is converted into the sulphide by heating it, with or without carbon, to a temperature of about 800°-950° C. in vapours of carbon bisulphide. Alternatively the magnesia may be mixed with carbon, for example in the form of coke or charcoal, the mixture introduced into the furnace and subjected at the requisite temperature to the action of sulphur vapours or sulphuretted hydrogen. The furnace in which the formation of the magnesium sulphide is effected may be heated electrically or in any other manner. Preferably the reaction mass is well mixed during the sulphidisation process in order to speed up the reaction and for this purpose the furnace employed may for instance be one of the rotary tube furnace type. The interior of the furnace must be kept free from moisture or air during the operation. After the sulphide has been formed it is then well mixed with the requisite amount of finely powdered calcium carbide and any desired flux, the admixture taking place in the reduction furnace itself. Thereupon at the high temperature prevailing suitably 1250° C., the sulphide is decomposed by the action of the calcium carbide with the formation of magnesium. The sulphur is obtained in the form of calcium sulphide from which it can be recovered by the action of superheated steam in the usual manner, the sulphuretted hydrogen first formed being incompletely oxidized by a combustion in air so as to produce elemental sulphur. The recovery of the sulphur from the calcium sulphide 50 can be expressed by the following equations:



But this recovery can also be carried out by the action of carbon dioxide as follows:



The present process has the advantage that the magnesium can be obtained at a temperature of 60 between 1200°-1250° C., but this temperature can be lowered if desired by carrying out the reactions under a reduced pressure.

Since the formation of the magnesium sulphide requires a considerably longer time than 65 the reduction to metal, these facts must be borne in mind and taken account of in arranging the details of the process so as to operate it as a continuous one.

When the magnesium sulphide is produced from 70 magnesia mixed with charcoal by the action of sulphur vapours, the reaction is effected by heating the mixture at about 950° C. This reaction may be expressed by the following equation:



If desired the magnesium oxide may be first of all treated with magnesium chloride,  $\text{MgCl}_2 \cdot 6\text{H}_2\text{O}$ , the product dried and thereafter mixed with coke and treated with sulphur vapours at the temperature above mentioned, whereby there is obtained 5 a mixture of magnesium sulphide and magnesium chloride, the presence of the latter being an advantage since it serves as flux for the subsequent calcium carbide treatment in the final stage of the process.

It may also be mentioned that products, such as sulphur or carbon bisulphide, employed in the present process in the formation of the magnesium sulphide can be recovered for reuse in the process.

Magnesium is finally produced from the magnesium sulphide or mixture of magnesium sulphide and magnesium chloride in the manner hereinbefore explained.

#### 15 EXAMPLE 2

##### *Production of magnesium from dolomite*

The first stage is the formation of magnesium sulphide. This is best effected by heating the dolomite at about 600°-800° C., in a furnace in 20 order to liberate the major part of the carbon dioxide from the double carbonate. There is thus obtained a mixture of calcium and magnesium oxides. The calcination of the dolomite can be effected either by directly heating it or by mixing 25 with it carbonaceous materials such as coke and heating the mixture to the requisite temperature. The carbon dioxide thus obtained can be collected and utilised for any industrial purposes, for example for the manufacture of "dry ice".

The mixture of calcium and magnesium oxides thus obtained is then subjected to treatment in the manner previously described for the conversion of the magnesia into sulphide, whereafter, by reduction of the latter with calcium carbide magnesium is obtained.

#### EXAMPLE 3

##### *Production of magnesium from magnesium sulphate*

The magnesium sulphate is first decomposed by heating it in the presence of carbon (such as coke) to a temperature of about 900° C., whereby carbon dioxide, sulphur dioxide, sulphur and magnesia are obtained. The magnesia so produced is 45 treated with magnesium chloride,  $\text{MgCl}_2 \cdot 6\text{H}_2\text{O}$ . If so desired the magnesium chloride can be replaced by hydrochloric acid gas, the requisite proportion of this latter being employed to form the oxy-chloride,  $\text{MgO} \cdot \text{MgCl}_2$ . The magnesium oxychloride in whichever way obtained is well dried and thereafter treated in the manner previously described so as to convert the oxide into the sulphide, a product of the composition  $\text{MgS} \cdot \text{MgCl}_2$  50 being obtained. This product is then treated with calcium carbide whereby metallic magnesium is obtained.

It will of course be understood that any other magnesium ores or salts can be treated according 60 to the general method herein described for the production of magnesium.

It will also be understood that the invention is not limited to the reduction of magnesium sulphide only, but that derivatives of magnesium sulphide, such as magnesium oxysulphide magnesium chloro-sulphide and mixtures thereof produced according to the present process, can be treated in the same manner with a carbide of an alkali earth metal, preferably with calcium carbide, for the production of magnesium.

Further, it may be mentioned that products such as sulphur or carbon bisulphide employed in the present process are recovered for reuse in the process.

I claim:

1. A process for the industrial production of magnesium from magnesium compounds which consists in first producing magnesium sulphide by the step of heating such magnesium compound with a reacting agent containing carbon and sulphur, in a non-oxidizing atmosphere free from moisture and air, and to a reacting temperature sufficiently high, namely, between about 800° and 1200° C., whereby to convert the bulk of the magnesium compound into magnesium sulphide; and thereupon reducing such magnesium sulphide, before its decomposition occurs, by the step of heating it in mixture with a reacting agent containing a carbide of another earth-alkali metal, in a non-oxidizing atmosphere free from moisture, air and nitrogen, and to a reacting temperature higher than that in the first reaction, namely, between about 1200° and 1600° C., whereby magnesium vapours are formed and distilled off for separate condensation.
2. A continuous process for the industrial production of magnesium from magnesium compounds which consists in a first stage in producing magnesium sulphide by the heating of such magnesium compound with a reacting agent containing carbon and sulphur, in a non-oxidizing atmosphere free from moisture and air, and to a reacting temperature well inside the range between 800° and 1200° C., whereby to convert the bulk of the magnesium compounds into magnesium sulphide; and in the succeeding stage reducing such magnesium sulphide, before its decomposition occurs, by the step of heating it in finely divided mixture with a reacting agent containing a carbide of another earth-alkali metal, in a non-oxidizing atmosphere free from moisture, air and nitrogen, and to a reacting temperature higher than that in the first reaction, namely, inside the range between 1200° and 1600° C., whereby magnesium vapours are formed and distilled off for separate condensation; while methodically removing byproducts including slag and replenishing the compounds and agents of said reactions.
3. The process as in claim 2 and wherein the second mentioned stage is performed with the assistance of a halide flux and at a temperature not greatly above 1200° C.
4. The process of claim 1 and wherein the first named reaction agent is a carbonaceous reducing agent in sulphur vapours.
5. The process of claim 1 and wherein the first

named reaction agent is a gaseous vaporized non-metallic sulphur compound.

6. The process of claim 1 and wherein the first named reaction agent is carbon bisulphide vapor.

7. A continuous process for the industrial production of magnesium from magnesium oxychloride which consists in first heating dry magnesium oxychloride with a reacting agent containing carbon and sulphur, in a non-oxidizing atmosphere free from moisture and air, and to a reacting temperature of about 950° C. more or less within the range between 800° and 1200° C., whereby to convert the bulk of the magnesium oxychloride into magnesium sulphide and magnesium chlorosulphide; and thereupon reducing these reaction products by the step of heating them in mixture with a reacting agent containing a carbide of another earth-alkali metal, in a non-oxidizing atmosphere free from moisture, air and nitrogen and containing a reducing gas, and to a reacting temperature between about 1200° and 1600° C., whereby magnesium vapours are formed and distilled off for separate condensation.

8. A continuous process for the industrial production of magnesium from calcined magnesite which consists in first producing magnesium sulphide by the step of heating such magnesite with a reacting agent containing carbon and sulphur, in a non-oxidizing atmosphere free from moisture and air, and to a reacting temperature of about 950° C., or more, whereby to convert the bulk of the magnesite into magnesium sulphide; and thereupon reducing such magnesium sulphide, before its decomposition occurs, by the step of heating it in powdered mixture with a reacting agent containing a carbide of another earth-alkali metal, in a non-oxidizing atmosphere free from moisture, air and nitrogen, and to a reacting temperature higher than that in the first reaction, whereby magnesium vapours are formed and distilled off for separate condensation.

9. A process as in claim 1 in which the reduction of the magnesium sulphide in the second step is effected by heating it with calcium carbide in an atmosphere of a non-oxidizing gas.

10. A process as in claim 1, in which the magnesium obtained from the reduction of the magnesium sulphide is distilled off, conducted away and condensed into a molten metal with which it is to be alloyed.

DANIEL GARDNER.